

Patented Apr. 19, 1927.

## UNITED STATES PATENT OFFICE.

STANLEY FOWLER, OF YORKSHIRE, AND EDWIN EDSER, OF LONDON, ENGLAND.

## LUBRICANT.

No Drawing. Application filed January 25, 1927, Serial No. 163,551, and in Great Britain March 24, 1925.

This invention comprises improvements in lubricants. The present application is in part a continuation of our prior United States application Serial No. 104,833, filed

5 April 26, 1926.

It has hitherto been proposed to employ as lubricants mixtures of lubricating oils with materials derived from the treatment of wool-fat and it has been emphasized that 10 the wool-fat employed should be neutralized and free of soaps. We have found, however, that it is not sufficient to render the wool-fat neutral and soap-free. Ordinary neutralized cholesterol preparations at normal 15 atmospheric temperatures yield a sediment when admixed with mineral hydrocarbons either immediately or after a time, the whole of the wool-fat thus not going into permanent solution in the oil. The sediment in general forms progressively with time and materially diminishes the value of the lubricant.

We have discovered that this sediment is due to impurities which can be removed, 25 for example by the process set forth in our United States Patent No. 1,610,854. This process consists essentially in the steps of first neutralizing a part of the free fatty acids in an aqueous mixture of the crude 30 wool-fat by addition of alkali in quantity insufficient to effect complete neutralization, removing the soaps produced, thereafter effecting further neutralization and removing the soaps produced by the further neutralization. 35 The neutralization of the free fatty acids present in the wool-fat is therefore effected in a plurality of stages. By so doing it has been found possible to prevent the formation of emulsions containing large quantities of wool-fat, as well as saponified material. The process also causes hydrolyzation 40 of esters insoluble in mineral oils which are present in the wool grease by the neutralization steps and these esters are removed with the soaps so that the product is freed 45 from esters as well as fatty acids and soaps. The product is, moreover, distinctly more transparent and waxy in character than wool-fats purified by solvent extraction processes. Wherever, in the claim, "purified 50 wool-fat" is mentioned it is to be understood that the product of the above described process is intended.

The presence of the specified impurities 55 can be detected by dissolving wool-fat in twice its own weight of benzene. Wool-fat

which is soluble to a non-turbid solution in the above-mentioned proportion of benzene at normal atmospheric temperatures has been found by us not to yield the aforesaid sediment or cloudiness when admixed with mineral-lubricating oils. The presence of a slight amount of a transparent separated colloidal body in the benzene solution after standing twenty-four hours may not indicate 65 detrimental impurities provided the solution is not turbid when initially prepared.

Moreover purified wool-fat suitable for use according to the present invention melts to a clear liquid free from turbidity if heated 70 and can be heated to 120° C. without frothing at the surface. If warmed and dissolved in one half of its weight of benzene and the warm liquid mixture is shaken no froth, or at most a quickly evanescent froth, is produced. Ordinary purified wool-fat yields a 75 froth when heated, is turbid when liquefied and gives turbid solutions. Our investigations have not enabled us to state with certainty the precise nature of the said impurities but they may be some kind of esters, for instance cholesterol esters.

According to the present invention, therefore, a lubricant is provided which consists essentially of a neutral hydrocarbon substantially non-volatile at normal atmospheric temperatures admixed with purified wool-fat which is soluble to a non-turbid solution in twice its own weight of benzene 80 at normal atmospheric temperatures.

The following is a description of one example of the preparation of a lubricant in accordance with the present invention:—

The wool-fat is first prepared in the manner set forth in our United States Patent 95 No. 1,610,854.

This purified wool-fat has the following partial analysis:—free fatty acid, less than 0.5% (calculated as oleic acid); ash, 0.1% (representing soaps and other impurities); 100 water, nil.

This material dissolves without turbidity in twice its weight of benzene and it will also be found to dissolve completely and permanently in mineral-lubricating oils.

The purified wool-fat is poured, while molten, into neutral mineral lubricating oil having a viscosity lying above 400 seconds Saybolt at 100° F. The temperature of the mixture may reach 50° C. owing to the heat of the wool-fat. The amount of oil 110 may vary but may be about three or more

times the amount of wool-fat. The product is a lubricant according to the present invention.

It is found that if the mineral oil has a viscosity above 400 seconds Saybolt at 100° F. and is used in about the proportions stated the product is suitable for general use in internal-combustion engines or the like. If a less liquid product is desired less mineral-oil may be used, or a thick mineral-grease, such as petroleum jelly may be used, as a thickening agent with the mixture of wool-fat and thin oil.

The product has valuable anti-corrosive properties as more fully set forth in our co-pending United States application Serial No. 130,100, filed August 18, 1926. Thus it has been found that the product will prevent rust on metallic surfaces to a degree beyond that capable of being obtained with other known preparations. Since it has non-corrosive properties and will adhere tenaciously to the surface and since it is also a good lubricant the thin layer of surface coating of this product need not be removed when the machines having their parts coated therewith are put into operation but the film may be left on the parts.

It has already been pointed out hereinabove that the wool-fat employed according to the present invention is completely

soluble in the mineral hydrocarbon oil used to mix with it. One advantageous result of this fact is that the wool-fat can be employed in the proportions needed to yield a lubricant of relatively high viscosity, whereas hitherto, with a view to reducing the tendency to sediment, the proportions of wool-fat have been in certain cases limited to the production of these lubricating oils of viscosity ranging from 200 to 400 seconds Saybolt at 100° F.

We claim:—

A lubricant consisting essentially of anhydrous wool-fat containing less than 0.5% of fatty acids calculated as oleic acid yielding less than 0.1% of ash, capable of dissolving to a clear solution without producing cloudiness or sediment in a mineral lubricating oil, and containing such small quantities of impurities insoluble in benzene at normal atmospheric temperatures as not to render a solution of the wool-fat in twice its weight of benzene turbid, such wool-fat being homogeneously admixed with a mineral lubricating-oil having a viscosity above 400 seconds Saybolt at 100° F.

In testimony whereof we affix our signatures.

STANLEY FOWLER.  
EDWIN EDSER.